

# UNITED STATES PATENT OFFICE.

THOMAS HAWKINS, OF BALMAIN, NEW SOUTH WALES, AUSTRALIA, ASSIGNOR TO POWERITE EXPLOSIVE COMPANY LIMITED, OF SYDNEY, NEW SOUTH WALES, AUSTRALIA.

## EXPLOSIVE.

1,202,712.

Specification of Letters Patent. Patented Oct. 24, 1916.

No Drawing.

Application filed November 11, 1915. Serial No. 60,914.

To all whom it may concern:

Be it known that I, THOMAS HAWKINS, a subject of the King of Great Britain and Ireland, residing at 7 Rowantree street, Balmain, in the State of New South Wales, Commonwealth of Australia, have invented certain new and useful Improvements in Explosives, of which the following is a specification.

10. This invention relates to an explosive for use in ordnance and small arms, and is devised with the object of providing an explosive compound having in a marked degree the following characteristics:—stability under varying conditions of storage, simplicity of manufacture, economy of production, safety in handling, and more particularly great power and cleanliness—that is to say the residue after firing is practically *nil*.
15. The explosive is compounded of the following four ingredients:—nitroglycerin, nitrocellulose, calcium picrate, and petrolatum; and in this regard bears a strong resemblance to the well known “cordite,” the difference being in the additional ingredient (calcium picrate) and in the proportions of those ingredients which are common to both. These features result in a great increase of explosive force as compared with cordite.
20. For the purpose of comparison, the percentage composition of my new explosive and of cordite are tabulated hereunder:—

*This invention. Cordite.*

|    |                                                       |       |        |
|----|-------------------------------------------------------|-------|--------|
| 35 | Nitroglycerin (prepared as<br>hereinafter described)  | 64.53 | 58.00  |
| 40 | Nitrocellulose (prepared as<br>hereinafter described) | 32.46 | 37.00  |
|    | Petrolatum                                            | 1.00  | 5.00   |
| 45 | Calcium picrate                                       | 2.00  | —      |
|    |                                                       | 99.99 | 100.00 |

In compounding this new explosive the nitroglycerin prepared by known and approved method is thoroughly washed (to remove all traces of free acid) in an alkaline solution composed of water 96 parts, borax 2 parts, sugar 1 part, and lime 1 to 2 parts; 50 it is then repeatedly washed in clear fresh

water. By this treatment a nitroglycerin is obtained which clears rapidly and which is stronger than ordinary nitroglycerin and safer to handle. The nitrocellulose is boiled in a vacuum apparatus for about 20 minutes 55 at a temperature not exceeding 100° C. in the said alkaline solution, and then subjected to cold running water for about two hours, after which it is pressed and dried in the usual manner. This treatment procures an 60 absolutely pure and neutral gun cotton which is not liable to change.

In 4517.32 grains of nitroglycerin treated in the manner above stated I dissolve as fully as possible 2272.68 grains of nitro- 65 cellulose treated as above stated and with the aid of a solvent (acetone) but without heat reduce them to a gelatinized condition. To this gelatinized or colloidal substance I add 140.00 grains of calcium picrate which 70 is soluble therein, and I intimately blend and incorporate them so as to form a homogeneous and uniform substance. Lastly when most of the acetone has evaporated I add 70.00 grains of petrolatum having a flash 75 point of not below 204.5° C. (400° F.) and not completely melting below 30.0° C. (86° F.), and continue the mixing for some time until the compound is of a suitable consistency to be cut into thin cords or strips 80 by suitable means as in the manufacture of cordite. After the adding of the petrolatum the mixing is performed on a table having preferably a surface of glass, porcelain, or the like, on which the compound is evenly 85 spread.

What I claim as my invention is:—

An explosive compound comprising approximately 64.53 per cent. of nitro-glyc- 90 erin, 32.46 per cent. of nitro-cellulose, 1 per cent. of petrolatum, and 2 per cent. of cal- cium picrate.

Signed at Sydney, New South Wales, Australia, this fifth day of October A. D. 1915.

THOMAS HAWKINS

Witnesses:

Wm. NEWTON,  
EMILY P. BARNETT.